

## UNITED STATES PATENT OFFICE

2,203,850

## CONVERSION OF HYDROCARBONS

Hans Tropsch, deceased, late of Chicago, Ill., by  
 Carl W. von Heimolt, administrator de bonis  
 non, Chicago, Ill., assignor to Universal Oil  
 Products Company, Chicago, Ill., a corporation  
 of Delaware

No Drawing. Continuation of application Serial  
 No. 37,342, August 22, 1935. This application  
 January 24, 1938, Serial No. 186,669

11 Claims. (Cl. 196—52)

This application is a continuation of co-pending application filed in the name of Hans Tropsch, Serial No. 37,342, filed August 22, 1935.

This invention relates particularly to the conversion of hydrocarbon fractions produced from naturally-occurring petroleums and particularly the distillate portions thereof, though the process may also be applied to analogous fractions produced in the primary distillation of more or less solid hydrocarbonaceous material such as coals, shales, lignites, etc.

More specifically, the invention is concerned with a process for converting a substantial portion of relatively heavy hydrocarbon fractions into lower boiling fractions suitable for use as motor fuel in automotive engines, the feature of the process which will be developed in more detail in the following specification being the employment of a particular class of compact materials for accelerating the catalytic decomposition reactions, so that more moderate temperatures and pressures may be used than those common to the majority of non-catalytic cracking processes.

In the ordinary cracking of heavy hydrocarbon fluids to produce economic yields of motor fuel, the conditions of operation in regard to temperature, pressure and time of exposure to cracking conditions are quite severe and the present day tendency is toward the use of conditions of increasing severity, since this seems to be the only way to meet the demand for motor fuel of high antiknock value. The use of temperatures of the order of 950° to 1100° F., with pressures of several hundred pounds per square inch, requires the use of very special metals adapted to withstand the strain without undue hazards, and it is obvious that the use of these severe conditions is attended with greatly increased expense in addition to greater danger.

Catalysts have seemed to offer the solution to the cracking problem in making possible the use of lower temperatures and pressures to accomplish the results obtainable at considerably higher temperatures and pressures without catalysts. However, in spite of a large amount of experimenting, but few catalysts have been developed which meet the requirements of low cost, resistance to poisoning influences and general ruggedness of structure, in addition to possessing the power to accelerate the cracking reactions in the desired directions. The better metal catalysts, such as nickel or cobalt, have a tendency to cause the splitting off of undue amounts of hydrogen and light gases in preference to fostering cracking reactions, and in addition are quickly ren-

dered inert when used with sulfur-containing oils on account of their conversion to sulfides which possess only low catalytic properties.

In one specific embodiment the present invention comprises the cracking or conversion of hydrocarbon distillates for the production of low boiling motor fuel fractions therefrom in the presence of catalysts comprising modified feldspars which have been treated for the removal of a substantial portion of their alkali metal and aluminum content and then caused to adsorb minor amounts of promoters from metal salt solutions.

As a result of extended investigations it has been found that catalysts of the character mentioned possess unusual value in cracking reactions. To assist in developing the character of the preferred catalysts, the following brief description of the feldspars as a mineral group is given:

The feldspars are ortho silicates of alkali and/or alkaline earth metals and aluminum, the alkali and alkaline earth metals being in iso-morphous mixtures. The general formula for the feldspar minerals is:  $(R, R') AlSi_3O_8$ , in which  $R$  represents an alkali metal, usually sodium or potassium, and  $R'$  represent an alkaline earth metal, usually calcium or barium, since the feldspars are quite uniformly characterized by the complete absence of magnesium and iron.  $R$  and  $R'$  may be considered collectively under the term "alkalinous" metal. The following table gives the names and formulas of the principal minerals of the feldspar group, these being taken from "A System of Mineralogy" by Dana, 6th edition, page 314.

## FELDSPAR GROUP

## a. Monoclinic section

|                 |                          |    |
|-----------------|--------------------------|----|
| Orthoclase      | $KAlSi_3O_8$             | 40 |
| Soda-orthoclase | $(K, Na) AlSi_3O_8$      |    |
| Hyalophane      | $(K_2, Ba) Al_2Si_4O_12$ |    |

## b. Triclinic section

|                 |                     |    |
|-----------------|---------------------|----|
| Microcline      | $KAlSi_3O_8$        | 45 |
| Soda-microcline | $(K, Na) AlSi_3O_8$ |    |
| Anorthoclase    | $(Na, K) AlSi_3O_8$ |    |

## Albite-anorthite series

|             |                  |    |
|-------------|------------------|----|
| Albite      | $NaAlSi_3O_8$    | 50 |
| Oligoclase  | $nNaAlSi_3O_8$   |    |
| Andesine    | $nCaAl_2Si_2O_8$ |    |
| Labradorite |                  |    |
| Anorthite   |                  |    |

The general characteristics of the feldspar

minerals are their crystallization in the monoclinic or triclinic systems; their cleavage in two similar directions at an angle of about 90°; their hardness, falling between 6 and 6.5; their specific gravity, falling principally between 2.55 and 2.75, and their colors, being white or pale shades of yellow, red or green.

According to the concept of the present invention, the naturally-occurring feldspar minerals, which are abundant and relatively cheap, are altered in both chemical and physical characteristics by the removal of a considerable proportion of their alkali metal and aluminum components and absorption of minor amounts of metal salts from aqueous solutions thereof, this combination of treating steps yielding catalytic material of markedly greater potency than the original feldspar or the intermediate material after the treatment for the removal of the alkali metals and aluminum. The general procedure for effecting the treatment of feldspars according to this process is given below:

1. The heating in the dry condition of proportioned mixtures of feldspar, lime and calcium chloride.

2. The washing of the treated feldspar particles from Step 1 to remove soluble material, principally sodium and potassium chlorides, along with part of the calcium chloride used as a reagent.

3. The further treatment of the partially altered feldspar with a mineral acid, followed by washing to remove aluminum, lime and calcium chloride.

4. The digestion of the treated feldspar with solutions of metal salts, principally those of aluminum and the heavy metals (those having a specific gravity of over 4), to effect the adsorption of small amounts of metal salts on to the more or less activated residue of the feldspar molecules.

5. The final calcination of the treated material to decompose at least a portion of the adsorbed salts to release acid radicals and remove water and form a certain amount of metal oxides which apparently act as promoters.

The following specific example of the preparation of an altered feldspar cracking catalyst is given to illustrate the general method:

Five hundred parts by weight each of finely ground orthoclase, lime, and calcium chloride were intimately mixed and heated for about 3 hours at a temperature of 1202° F. (650° C.). The partially fused mix was allowed to cool, pulverized, and washed with about 2 volumes of water. By this washing step, potassium chloride was extracted, this being recoverable on evaporation of the wash water. The washed material was then digested with about 4 volumes of a 10 per cent hydrochloric acid, after which the remaining insoluble material was washed with water first by decantation and later by filtering until substantially no chlorides were present in the wash water. The treated feldspar particles were then added to an aqueous solution consisting of 33.3 parts by weight of hydrated aluminum sulfate

( $\text{Al}_2(\text{SO}_4)_3 \cdot 18\text{H}_2\text{O}$ )

in about 3,000 parts by weight of water, and the suspension was then digested at the boiling point of the solution, using a reflux condenser for a period of about 18 hours. The particles were again washed by decantation and later by filtering until the wash water contained no sulfates. By this final treating step a small amount of aluminum salt was apparently adsorbed, probably in the form of a partially hydrolyzed sulfate

which was then decomposed to oxide by heating the treated feldspar for some time at a temperature of about 1000° F.

Following the above general procedure, it is possible to prepare a considerable number of alternative catalysts in which salts of other metals than aluminum, for example, iron, nickel, cobalt, chromium, molybdenum, tungsten, zinc, cadmium, copper etc., have been adsorbed on the preliminarily treated feldspars. Such modified feldspars all exhibit a considerably improved catalytic effectiveness when compared with the original feldspar mineral, but the effect of the final treatment by different metal salts upon the catalytic properties of various "dealkalized" feldspars varies considerably, and it is not to be inferred that the different alternative catalysts which may be produced by the general procedure outlined are in any sense equivalents among themselves in any one cracking reaction or in different cracking reactions. Thus the catalysts may vary from being specific for breaking the carbon-to-carbon bond or cracking to carbon or hydrogen.

It is comprised within the scope of the invention to treat any representative of the feldspar group of minerals first for the removal of a portion or substantially all of the alkali metal content, second for the removal of a portion or substantially all of the aluminum content, and then with different metal salts either single or in combination to further enhance their catalytic properties. Practically any soluble salt may be employed such as a sulfate, chloride, or nitrate although suitable modifications of concentration, time of treatment with the solution, and final calcination of the treated feldspar particles will obviously be necessary. It has been definitely determined that the preliminarily treated feldspars are not zeolytic in character in that the effect of treating with the aqueous solutions of metal salts is not to introduce equivalent metals in place of the removed alkali metals. Analyses of the feldspars after treatment with metal salt solutions indicate that there is no stoichiometric relationship between the amount of alkali metals removed and the amount of metal salts adsorbed, that the metal salts are held by adsorptive and not by the usual volume forces and that their oxides produced by calcination act as catalyst promoters. The phenomenon of promoter catalysis is none too well understood at the present time and the present instance is merely cited as one manifestation of the general law.

By the use of catalysts of the present character, it is possible to effect cracking of hydrocarbon distillates which are more or less readily vaporizable at temperatures and pressures considerably lower than those necessary for producing motor fuel fractions of a required antiknock value without the use of catalysts. As stated previously, the common range of cracking temperatures chosen to produce premium motor fuel fractions from heavy petroleum distillates varies from about 950° to 1100° F. and the pressure employed under these conditions varies from about 100 to 500 pounds per square inch. When the present type of catalysts are employed, it is seldom necessary to use temperatures over 950° F.; e. g., a range of 850° to 950° F. is satisfactory; and further, it is only necessary to employ atmospheric or very slightly super-atmospheric pressures. The increased rate of cracking makes possible the use of the same throughput of oil for an apparatus of a given volumetric capacity that was possible

at high super-atmospheric pressure, and, secondly, permits the use of much thinner tubes and reaction chambers, with considerably reduced costs.

The preferred method of operation when using catalysts of the present character is to heat and vaporize the oil to be cracked during passage through a tubular heating element wherein the temperature is raised to the best point for contact with the catalyst and then pass the vapors downwardly through a bed of granular catalyst particles contained in a vertical cylindrical treating chamber to effect the cracking reactions. The size of the particles which are most economically employed will vary somewhat but is usually comprised within the range of 4 to 20 mesh. After the cracked materials leave the catalyst chamber, they are subjected to fractionation to separate fixed gases, gasoline boiling range distillates, fractions suitable for recycling, and materials which are generally unsuitable for further cracking. It is generally preferable to operate the cracking process when using the present type of catalyst in such a way that there is a limited conversion per pass and if desired the recycle fractions may be subjected to further catalytic decomposition in contact with different catalysts and at different temperatures, or under conditions better suited for their conversion.

The following example is given to show the general character of the results obtainable by the use of catalysts falling within the general class covered by the present invention. The data given are typical but are not introduced for the purpose of correspondingly limiting the scope of the invention, since other examples of a generally similar character are available.

An orthoclase feldspar was treated for the removal of alkali metals and aluminum and later subjected to treatment with aluminum sulfate solution to permit the absorption of aluminum sulfate as described in a preceding paragraph.

The following data are introduced to indicate in a general way the effect of the treatment on the chemical composition of the original feldspar. The first column of figures shows the analysis of the original orthoclase without considering any water content. The second column shows the calculated composition which would correspond to the orthoclase if all alkali metals were removed and replaced by alumina. A third column shows the actual analysis of the material formed as a result of the preliminary treatment for the removal of alkali metals and part of the aluminum followed by the treatment with aluminum sulfate solution and the final calcining, leaving out the water content in all instances.

| Constituent                    | 1<br>Ortho-clase | 2<br>Replaced<br>orthoclase<br>(calculated) | 3<br>Treated<br>orthoclase |
|--------------------------------|------------------|---------------------------------------------|----------------------------|
| SiO <sub>2</sub>               | 64.8             | 72.6                                        | 89.1                       |
| Al <sub>2</sub> O <sub>3</sub> | 18.2             | 27.4                                        | 7.2                        |
| K <sub>2</sub> O               | 17.0             | 0.0                                         | 1.9                        |
| Undetermined                   | 0.0              | 0.0                                         | 1.8                        |

Analyses of gases evolved during the calcining step showed oxides of sulfur, indicating that the originally adsorbed aluminum sulfate had decomposed to aluminum oxide.

Using the above prepared catalyst in a fineness of 6 to 10 mesh in a vertical cylindrical catalyst chamber the vapors of a Mid-Continent gas oil were passed downwardly therethrough at a temperature of 932° F. and a slight superatmospheric

pressure to ensure proper flow through the reactor and succeeding fractionating equipment. The rate of feed of the gas oil was regulated so that the initial conversion per pass was of the order of 25 per cent, based on 400° F. end-point gasoline production. The recycle stock falling within the same proximate range as the original gas oil was separately re-cracked in contact with the same type of catalyst at the same temperature but at a somewhat reduced feed rate, the products from the cracking zone operating upon the recycle stock being introduced into a common fractionator with the products from the primary cracking operation.

The following table shows the principal significant data obtained as the result of an extended period of operation:

#### CRACKING RESULTS

|                                     |    |    |
|-------------------------------------|----|----|
| Per cent 400° F. end-point gasoline | 52 | 20 |
| Per cent Diesel fuel                | 20 |    |
| Per cent residuum                   | 20 |    |
| Gas loss                            | 8  |    |

#### PROPERTIES OF GASOLINE

|                       |           |     |
|-----------------------|-----------|-----|
| Gravity               | °A. P. I. | 56  |
| Initial boiling point | °F.       | 100 |
| 50% over at           | °F.       | 275 |
| End boiling point     | °F.       | 399 |
| Octane number         | 82        | 30  |

The practical value of the present invention can be readily seen from a consideration of the above figures, since it is fairly well known that gasoline having an anti-knock rating corresponding to over 80 octane number is not producible in the yield indicated under non-catalytic cracking conditions and particularly at low pressure. The gasoline produced as a result of the above run was readily stabilized by the addition of small amounts of commercial inhibitors which preserved its olefinic content from deterioration over a sufficient time to permit its storage under average refinery conditions.

The foregoing specifications and single example are sufficient to disclose the character of the present invention and its practical value though neither section is intended to be unduly limiting upon its proper scope.

#### What is claimed is:

1. A hydrocarbon oil conversion process which comprises contacting the oil at cracking temperature with a modified feldspar produced by removing from feldspar at least a part of its alkalinous base and aluminum content, adsorbing on the residual portion of the feldspar, from aqueous solution, a salt of a metal whose oxide is catalytic and then calcining to convert said salt to the catalytic metal oxide supported on the residual portion of the feldspar.

2. A hydrocarbon oil conversion process which comprises contacting the oil at cracking temperature with a modified feldspar produced by removing from feldspar at least a part of its alkalinous base and aluminum content, treating the residual portion of the feldspar with an aqueous aluminum salt solution to adsorb aluminum salt thereon and then calcining to convert the adsorbed salt to aluminum oxide supported on the residual portion of the feldspar.

3. A hydrocarbon oil conversion process which comprises subjecting the oil to cracking conditions in the presence of a catalytic metal oxide supported on a feldspar whose alkalinous base and aluminum content has been removed at least in part.

4. A hydrocarbon oil conversion process which comprises subjecting the oil to cracking conditions in the presence of aluminum oxide supported on a feldspar whose alkalinous base and aluminum content has been removed at least in part.
5. A hydrocarbon oil conversion process which comprises subjecting the oil to cracking conditions in the presence of iron oxide supported on a feldspar whose alkalinous base and aluminum content has been removed at least in part.
6. A hydrocarbon oil conversion process which comprises subjecting the oil to cracking conditions in the presence of nickel oxide supported on a feldspar whose alkalinous base and aluminum content has been removed at least in part.
7. A process for producing gasoline from hydrocarbon oils heavier than gasoline which comprises subjecting the heavier oil to cracking conditions in the presence of a modified feldspar produced by removing from feldspar at least a part of its alkalinous base and aluminum content, treating the residual portion of the feldspar with an aqueous aluminum sulfate solution to adsorb aluminum sulfate thereon and then calcining to convert the adsorbed sulfate to aluminum oxide supported on the residual portion of the feldspar.
8. The process as defined in claim 1 further characterized in that said metal is iron.
9. The process as defined in claim 1 further characterized in that said metal is nickel.
10. A process for the conversion of hydrocarbon distillates to produce lower boiling hydrocarbons therefrom suitable for use as motor fuels, which comprises subjecting the vapors of said

hydrocarbon distillates at a conversion temperature of the order of 850-1000° F. and at substantially atmospheric pressure to contact with granular catalytic materials produced by heating feldspars with calcium oxide and calcium chloride mixtures followed by washing for the partial removal of alkalinous bases and aluminum, subjecting said treated feldspars to further treatment with solutions of metal salts to permit adsorption of said salts, and further drying and calcining said treated feldspars to volatilize a substantial portion of the acid radicals of said salts and leave residual compounds which function as catalysts.

11. A process for the conversion of hydrocarbon distillates to produce lower boiling hydrocarbons therefrom suitable for use as motor fuels, which comprises subjecting the vapors of said hydrocarbon distillates at a conversion temperature of the order of 850-1000° F. and at substantially atmospheric pressure to contact with granular catalytic materials produced by heating feldspars with calcium oxide and calcium chloride mixtures followed by washing for the partial removal of alkalinous bases and aluminum, subjecting said treated feldspars to treatment with solutions of heavy metal salts to permit adsorption of said salts, and further drying and calcining said treated feldspars to volatilize a substantial portion of the said acid radicals of said salts, and leave residual compounds which function as catalysts.

CARL W. VON HELMOLT,  
Administrator de Bonis Non Vitae Will Annexed 35  
of the Estate of Hans Tropsch, Deceased.